

## 1

2,760,999

## REFORMING OF NAPHTHA

Alex G. Oblad, Springfield, and Heinz Heinemann, Drexel Hill, Pa., assignors to Houdry Process Corporation, Wilmington, Del., a corporation of Delaware

No Drawing. Application November 30, 1950,  
Serial No. 198,468

2 Claims. (Cl. 260—668)

The present invention relates to the treatment of hydrocarbon distillates boiling approximately in the range of gasoline and is particularly concerned with reforming such distillates under the influence of selective catalysts and particular conditions favoring improvements in quality of the product including upgrading of the anti-knock properties thereof.

Among the objects of the invention is the provision of an improved reforming process wherein high yields of gasoline of desired enhanced octane quality are obtained, while minimizing the occurrence or extent of such other accompanying reactions, such as cracking, which tend to produce coke and low molecular weight hydrocarbon gases, at the expense of desired gasoline yields.

In previous known processes for upgrading gasoline and naphtha fractions, involving treatment at superatmospheric pressure and in the presence of added hydrogen, catalysts have been employed having the property of promoting dehydrogenation reactions, the best known being molybdenum oxides on activated alumina. While under the conditions employed in these previous processes dehydrogenation of naphthenes present in the gasoline charged to reforming does take place, other simultaneous reactions occur to substantial extent, including cracking of parts of the charge, resulting in the formation of significant quantities of low molecular weight hydrocarbon gases accompanied by deposition of coke in sufficient amounts to limit the practical on-stream operating period to about 4-8 hours, followed by regeneration of the catalyst. The reported butane-free gasoline yields from such processes are in the order of about 70-80% by volume of the charge. In other related processes conditions were employed to dehydrogenate selected narrow cuts of naphthenic materials to aromatic hydrocarbons, operating under conditions obtaining lower conversion of the charge per pass, and generally at higher pressures (up to about 50-70 atmospheres) than in the previously described process. In these processes operating at lower conversion levels longer on-stream periods of up to several days or more might be possible, requiring as much as about 20-24 hours for regeneration of the coke produced. Reformed products high in aromatic content are stated to be obtained, but the overall gasoline yields are not substantially better than those obtained in the previously described processes carried out at lower pressure.

In accordance with the present invention, naphthenes in gasoline and naphtha fractions, are selectively converted to aromatics under conditions disfavoring accompanying production of undesirable side products such as coke and gas. This desirable result is brought about by carrying out the reforming process under selected conditions and in the presence of catalysts which selectively promote dehydrogenation reactions and have little or no initial or potential tendency to promote cracking or polymerization reactions. More particularly, the selected reaction conditions include temperatures of 850-975° F. and preferably not above 950° F., pressures of about 400-1000 pounds per square inch, and liquid space rates (vol. oil/

## 2

hr./vol. cat.) of 1 or more, preferably at least 2. The selected catalysts employed are characterized by the properties of being capable of dehydrogenating methylcyclohexane to aromatics under fixed operating conditions while being incapable of significantly converting normal heptane under the same conditions.

Among the catalysts that can be employed in the process of the invention there are included noble metals of the platinum-palladium group supported on non-acidic carriers having no significant cracking activity, such as 0.1 to 2% Pt or Pd on MgO or on silica or titania gel; molybdenum oxides supported on inactive or inactivated carriers such as on silica gel, or on alumina specially treated to inactivate the cracking-promoting function thereof; 7.0 to 15.0% MoO<sub>3</sub> by weight of the catalyst is generally satisfactory. The selectivity of various catalysts can be tested by their separate effects on conversion of heptane and of methylcyclohexane under standardized conditions. In the following tabulation there are compared typical results obtained with catalysts of the invention as opposed to catalysts having significant cracking activity, such as 10% MoO<sub>3</sub> on alumina, in the conversion of the stated hydrocarbons at a temperature of 950° F. under a pressure of 600 p. s. i. g., feeding the oil at a liquid space rate of 2 (vol./hr./vol.), 3 mols of hydrogen being added with the charge.

TABLE 1

| Catalyst          | Pt—MgO<br>MoO <sub>3</sub> on inact.<br>Al <sub>2</sub> O <sub>3</sub> | MoO <sub>3</sub> —Al <sub>2</sub> O <sub>3</sub> |                                      |
|-------------------|------------------------------------------------------------------------|--------------------------------------------------|--------------------------------------|
|                   |                                                                        | Charge                                           | Yields (wt. percent charge) per pass |
| Methylcyclohexane | Aromatics.....                                                         | 80.....                                          | 86.....                              |
|                   | Other Prod.<br>(gas, etc.).....                                        | <5.....                                          | 10 to 10+.....                       |
| N-Heptane         | Aromatics.....                                                         | 5 (or less).....                                 | 12-16.....                           |
|                   | Other Prod.<br>(incl. gas).<br>Unconverted.....                        | <10.....<br>Circa 85-90.....                     | >50.....<br>30-35.....               |

Since by the process of the invention cracking is minimized, the quantity of low molecular weight gases produced is quite small and incremental coke deposition, if any, is so low that periodic regeneration of the catalyst is not necessary, or will be used only at infrequent intervals following an on-stream period going up to several weeks or more.

The reforming process of the invention is applicable to the treatment of various naphtha charge stocks containing naphthenes of the hydroaromatic type, including catalytically cracked distillates as well as straight run gasoline and naphthas and distillates from thermal cracking. An important application of the invention is in the treatment of gasoline and naphtha fractions derived from hydrogenative processes such as hydrogenative cracking and destructive hydrogenation, which fractions are generally characterized by a high naphthene content and low octane rating.

As pointed out in the copending application Serial No. 198,469, filed of even date herewith, and now abandoned, in the case of the noble metal catalyst, it is important that the support or carrier have a surface area adapted to extensive and uniform distribution of the active metal thereon and be free from components imparting acidity to the carrier; acidity can be measured by ability of the mass to chemisorb quinoline or other organic bases. Magnesium oxide is a preferred material for use as a carrier since it is relatively cheap and abundant, is slightly basic, and can be obtained or prepared in forms having the desired surface characteristics; both the light as well as the heavy forms of magnesia may be employed as well as the product obtained by simple precipitation by alkaline

medium of soluble magnesium salts, followed by drying.

The Pt or alternative metal component is employed generally in proportions of from about 0.1 to 2.0% by weight of the carrier (water free basis), and preferably in proportions of about 0.4-1% by weight thereof. Palladium and other noble metals of the platinum and palladium group or combinations of these are also suitable, but not necessarily with equal results. The hydrogenative metal component can be deposited in or on the carrier by impregnating the latter with an aqueous suspension of the metal oxide followed by reduction thereof to the free metal, or by dipping the carrier in soluble salts or other soluble compounds of the metals and decomposing the same to free metal or oxide. Thus, the magnesia in the form of pellets or granules of desired size may be dipped in a solution of chloroplatinic acid or chloroplatinous acid of suitable concentration to provide the desired quantity of Pt, then dried and decomposed by heating or reduction with hydrogen or by treatment with soda under reducing conditions. Palladium may be deposited by impregnation of the magnesia carrier with  $PdCl_2$  solution in suitable concentration followed by decomposition thereof directly to the metal, or to the oxide with subsequent reduction. Conversion of the oxides to free metal, if necessary, can be readily effected by reduction with hydrogen or other reducing agents in vapor form.

The deposition of the noble metal on silica or titania gel can be carried out generally in the manner already described for deposition thereof on magnesia carriers.

The molybdena-containing catalysts can be prepared by dipping the inactive or inactivated support in a solution of a soluble molybdenum salt, such as ammonium molybdate, and decomposing the salt to the oxide. The inactivation of supports such as alumina, including so-called activated and gamma alumina, is effected by treating the support with an alkaline earth compound, particularly with a magnesium or calcium salt in quantities effecting deposition of equivalent of 0.1 to 2% by weight of the alkaline earth oxide in the carrier. The deposition of the alkaline earth oxide in the carrier is effected prior to treatment with the molybdenum compound to obtain catalysts having the desired properties specified. It is also important that the alumina support, before or after deposition of the molybdenum compound be not heated to high temperatures or otherwise treated to cause transformation thereof to beta forms of alumina. Also suitable for deactivating the alumina support as to cracking function, but not necessarily with equal quantitative effect, are alkali metal oxides particularly sodium oxide. These can be incorporated in the alumina in the same manner as the alkaline earth metal oxides described above, and in about the same proportions.

#### Example I

Heavy magnesia powder (Merck #1478) was hydrated by agitation in water overnight then filtered. The filter cake was made into an extrudable mix by adjustment of water content (mixing wet and dried filter cake), a small amount of methyl cellulose added as plasticizer, and the

mixture extruded through dies into strands and cut into cylindrical pellets. The wet pellets were dried at temperatures not in excess of  $240^{\circ}$  F., ground to powder and dipped in aqueous chloroplatinic acid containing 1.5 times the required amount of Pt, employing about 56 milliliters of liquid per 100 grams of  $MgO$ . Excess liquid was filtered off and the powder oven dried, then heat treated in a muffle furnace for two hours at  $1000^{\circ}$  F. to drive off HCl. The powder was formed into pellets with addition of 5% corn oil and hardened by further heat treatment in air at  $1050^{\circ}$  F. for 2 hours.

A number of catalysts differing in Pt content were thus prepared including the following: 1.2% Pt on  $MgO$  by impregnating with an aqueous solution containing 54.5 grams  $H_2PtCl_6 \cdot 6H_2O$  per liter, and 0.6% and 0.4% Pt on  $MgO$  using solutions containing respectively 27 and 18 grams of  $H_2PtCl_6 \cdot 6H_2O$  per liter.

The several catalysts were treated with a flowing stream of hydrogen before being contacted with the hydrocarbon charge.

The following table illustrates a number of runs carried out with the above catalysts under the different operating conditions specified:

TABLE 2

[Catalyst 1.2% Pt on  $MgO$ .]

| Charge                                   | East Texas Naphtha (B. R. 190-370° F., 53.4° API) | East Texas Naphtha (B. R. 240-352° F., 53.3° API) |
|------------------------------------------|---------------------------------------------------|---------------------------------------------------|
| Paraffins, wt. percent                   | 30                                                | 41                                                |
| Olefins, wt. percent                     | 0                                                 | 0                                                 |
| Naphthenes, wt. percent                  | 48                                                | 45                                                |
| Aromatics, wt. percent                   | 13                                                | 14                                                |
| Octane Nos.:                             |                                                   |                                                   |
| CFR-R Clear                              | 51.2                                              | 57.6                                              |
| +3 cc. TEL                               | 76.6                                              | 72.4                                              |
| Operating Conditions:                    |                                                   |                                                   |
| Pressure, p. s. i. g.                    | 600                                               | 600                                               |
| Temp., °F.                               | 950                                               | 950                                               |
| LSV, vol./hr./vol.                       | 2                                                 | 2                                                 |
| H <sub>2</sub> /oil ratio                | 3                                                 | 6                                                 |
| Yields (percent of charge):              |                                                   |                                                   |
| Gasoline (C <sub>5</sub> +) vol. percent | 94.5                                              | 92.8                                              |
| C <sub>4</sub> , vol. percent            | 3.9                                               | 3.4                                               |
| Dry Gas, wt. percent                     | 1.4                                               | 3.0                                               |
| Coke, wt. percent                        | 0.2                                               | 0.2                                               |
| Octane Nos.:                             |                                                   |                                                   |
| CFR-M Clear                              | 61.4                                              | 60.8                                              |
| CFR-R Clear                              | 72.4                                              | —                                                 |
| CFR-R+3 cc. TEL                          | 87.5                                              | —                                                 |
| Paraffins, wt. percent                   | 37                                                | 42                                                |
| Olefins, wt. percent                     | 3                                                 | 2                                                 |
| Naphthenes, wt. percent                  | 23                                                | 19                                                |
| Aromatics, wt. percent                   | 37                                                | 36                                                |

It will be seen from the above table that at temperature of  $1000^{\circ}$  F. as compared with the runs at  $950^{\circ}$  F. significant cracking has begun to take place as evidenced by considerably increased quantities of C<sub>4</sub> and dry gas produced, comparatively high coke deposition, and reduction in paraffins by conversion.

The effect of change in space rate will be apparent from the runs in the following table showing results obtained charging the same naphtha feed. Also reported are several runs with catalyst of lower Pt content.

TABLE 3

[Charge: East Texas Naphtha (B. R. 240-352° F., API 53.3).]

| Catalyst—Percent Pt on $MgO$         | 1.2   | 1.2  | 0.6     | 0.4   |
|--------------------------------------|-------|------|---------|-------|
| Operating Conditions:                |       |      |         |       |
| Pressure, p. s. i. g.                | 750   | 600  | 600     | 600   |
| Temp., °F.                           | 950   | 950  | 950     | 950   |
| LSV, Vol./hr./vol.                   | 0.5   | 4    | 2       | 2     |
| H <sub>2</sub> /oil ratio            | 3     | 5    | 3       | 3     |
| Period, Min.                         | 0-240 | 0-30 | 150-180 | 0-120 |
| Yields (Percent Chg.):               |       |      |         |       |
| Gaso (C <sub>5</sub> +) vol. percent | 83.5  | 94.5 | 9.41    | 93.4  |
| C <sub>4</sub> , Vol. percent        | 11.5  | 1.6  | 1.8     | 2.9   |
| Dry gas, Wt. percent                 | 4.2   | 2.7  | 2.9     | 2.0   |
| Coke, Wt. percent                    | 1.1   | 0.02 | 0.02    | 0.1   |
| Octane Nos.:                         |       |      |         |       |
| CFR-R Clear                          | 82.8  | 69.4 | 71.5    | 73.1  |
| +3 cc. TEL                           | 93.7  | 85.6 | 87.8    | 87.8  |

From the foregoing results it appears that at space velocities below 1, cracking is commencing to take place to significant extent as evidenced by increase in dry gas and C<sub>4</sub>'s and notable coke depositions. At the preferred conditions of operation, it will also be observed, there is no significant change in catalyst properties, with increasing time on stream the yields remaining substantially constant.

*Example II*

Commercial activated-alumina tablets (Harshaw) were treated with 20% magnesium chloride (MgCl<sub>2</sub>) solution, using about 5 liters solution per kilogram of alumina, then washed free of chlorides and dried. The dried product was treated for thirty minutes with a solution of ammonium molybdate (calculated to deposit 10% MoO<sub>3</sub> on the alumina) containing about 270 grams MoO<sub>3</sub> per liter of water, in the proportions of about 400 milliliters solution per kilogram of alumina. The treated product was drained, dried, and heat treated at 1050° F. for two hours. Before being placed on stream, hydrogen was passed over the catalyst to reduce the molybdena to lower valence forms. The final catalyst contained 0.28% MgO.

The catalyst thus prepared was employed in reforming East Texas naphtha with the following results:

TABLE 4

[Charge: East Texas naphtha (B. R. 240-352° F., API° 53.3). Catalyst: MoO<sub>3</sub> on magnesia-treated alumina.]

| Operating conditions:                 | 600  | 600  | 750  | 750  |
|---------------------------------------|------|------|------|------|
| Pressure, p. s. i. g.                 | 600  | 600  | 750  | 750  |
| Temp., °F.                            | 950  | 950  | 950  | 950  |
| LSV (vol./hr./vol.)                   | 2    | 4    | 2    | 0.5  |
| H <sub>2</sub> : oil ratio            | 3    | 5    | 3    | 3    |
| Yields:                               |      |      |      |      |
| Gaso. (C <sub>5</sub> +) vol. percent | 86.5 | 91.3 | 88.8 | 76.4 |
| C <sub>4</sub> , vol. percent         | 8.1  | 4.4  | 7.2  | 17.4 |
| Dry Gas, wt. percent                  | 4.1  | 3.2  | 3.8  | 6.9  |
| Coke, wt. percent                     | 0.4  | .007 | 0.6  | 0.7  |
| Octanes:                              |      |      |      |      |
| CFR-R clear                           | 85.3 | 75.0 | 79.5 | 89.8 |
| +3 cc. TEL                            | 95.4 | 88.4 | 93.2 | 97.4 |

It will be seen from the above table that at space rates below 1 there is evidence of increased cracking as shown by considerable increase in C<sub>4</sub> and dry gas. By increasing temperature to above 975° F. as to about 1000° F., it was observed with the molybdena containing catalysts as well as with the noble metal catalysts, that there is a notable increase in cracking, obtaining yields and distribution of products similar to those obtained at the reduced space rates.

We claim as our invention:

1. The method of selectively dehydrogenating naph-

thenic hydrocarbons in a hydrocarbon fraction boiling approximately in the range of gasoline with concomitant formation of minimized quantities of normally gaseous hydrocarbons, coke and other cracked products which comprises contacting said hydrocarbon fraction with a nonacidic catalyst consisting essentially of 0.1 to 2% of noble metal from the group consisting of platinum and palladium deposited in a nonacidic dried gel carrier from the group consisting of silica gel and titania gel, said contacting of the hydrocarbon fraction with the catalyst being in the presence of several mols of added hydrogen per mol of hydrocarbon at a temperature within the range from about 850° F. to about 975° F. at a pressure within the range of from about 400 lbs. per sq. in. to 1000 lbs. per sq. in. at a space velocity within the range from about 1 to about 6 liquid volumes of hydrocarbon per hour per volume of catalyst, whereby substantially all of the methylcyclohexane content of said hydrocarbon fraction is converted substantially completely to toluene and whereby the normal heptane content of said fraction is recovered substantially completely as normal heptane.

2. The method of selectively dehydrogenating naphthenic hydrocarbons in a hydrocarbon fraction boiling approximately in the range of gasoline with concomitant formation of minimized quantities of normally gaseous hydrocarbons, coke and other cracked products which comprises contacting said hydrocarbon fraction with a catalyst consisting of 0.1 to 2% platinum in a nonacidic titania gel in the presence of about 5 mols of added hydrogen at a temperature of about 950° F. at a pressure of about 600 lbs. per sq. in. at a space velocity of about 4 liquid volumes of hydrocarbon fraction per hr. per volume of catalyst whereby the methylcyclohexane content of said fraction is converted substantially completely to toluene and whereby the normal heptane content of said fraction is recovered substantially completely as normal heptane.

References Cited in the file of this patent

UNITED STATES PATENTS

|    |           |                 |               |
|----|-----------|-----------------|---------------|
| 40 | 2,285,727 | Komarewsky      | June 9, 1942  |
|    | 2,373,674 | Crawford et al. | Apr. 17, 1945 |
|    | 2,409,382 | Peck            | Oct. 15, 1946 |
|    | 2,409,695 | Laughlin        | Oct. 22, 1946 |
| 45 | 2,411,726 | Holroyd et al.  | Nov. 26, 1946 |
|    | 2,479,110 | Haensel         | Aug. 16, 1949 |
|    | 2,550,531 | Ciapetta        | Apr. 24, 1951 |

OTHER REFERENCES

Komarewsky et al.: Oil and Gas Journal, pages 90, 91, 92, 93 and 119 (5 pages), June 24, 1943.